

## UNITED STATES PATENT OFFICE

2,089,939

## ALLOY

Jesse O. Betterton, Metuchen, and Albert J. Phillips, Plainfield, N. J., assignors to American Smelting and Refining Company, New York, N. Y., a corporation of New Jersey

No Drawing. Application May 2, 1936,  
Serial No. 77,614

3 Claims. (CL. 75—166)

In the production of various commercial grades of lead, the presence of bismuth as an objectionable impurity has been long recognized and generally accepted in the industry. The presence of such bismuth has been regarded, however, as a rather necessary evil in many forms of commercial leads, in view of the presence of such element in the raw materials from which the lead is derived. Lead ores from many localities contain substantial amounts of bismuth which is carried on through the reduction of the ores and is present in varying amounts in the commercial forms of lead which are produced from such sources.

When present in commercial lead in the amounts usually associated with the lead, it is generally recognized that the presence of this bismuth adversely influences certain of the properties of the lead with particular reference to its rate of corrosion toward sulphuric acid, and the reduction in creep strength of the lead. Because of these properties, lead containing substantial amounts of bismuth, even as low as in the neighborhood of 0.1% has been accepted as being unsuitable for purposes where high resistance to sulphuric acid corrosion, as, for example, in the manufacture of the lead chambers customarily used in the production of sulphuric acid, and also in the production of cable sheaths where a high creep resistance is desirable.

In view of these facts, it has become the practice to treat such leads with suitable debismuthizing agents for the purpose of eliminating the bismuth content, thereby removing the source of the objectionable properties above referred to, it having been accepted for many years that a bismuth-free lead-containing copper in which the copper content ranges from 0.04 to 0.08% is the standard acid corrosion-resisting lead alloy.

It has been discovered that the corrosion resistance of this alloy is due to the fact that the lead becomes coated with a protective layer of basic lead sulphate when exposed to sulphuric acid, which coating prevents further contact between the lead and the sulphuric acid.

This coating will form, of course, regardless of the presence or absence of bismuth in the lead being exposed; but it is believed that where the bismuth is present in substantial amounts, for instance around 0.1% and over, the reduction in the creep resistance of the lead will cause a continuous deformation of this protective coating, producing breaks in the same, so that the acid may continuously gain access to fresh metal so that the corrosion will proceed notwithstanding

the presence of the basic lead sulphate referred to above. In the case of the bismuth free lead-copper alloys mentioned above, there is high creep resistance, with consequent elimination of any appreciable deformation of this protective coating. 5

In accordance with the present invention, there is produced an improved corrosion resisting lead alloy, which exhibits substantially improved corrosion-resisting properties over the usual lead alloy compositions employed for sulphuric acid work. 10

The present improved composition is based upon the discovery that the low creep resistance manifested by bismuth-containing leads is due not 15 to bismuth alone, but to the presence in the lead of other constituents also present as the impurities therein, which act in a cumulative manner to decrease the resistance to creep and to corrosion.

It has been demonstrated, for example, that 20 the presence of silver, which is a very common contaminant of lead, very substantially reduces the creep resistance of the lead, and also increases the corrosion rate of the lead in sulphuric acid. Other common constituents frequently associated with lead which act in a similar manner are zinc, antimony, tin and arsenic. 25

In connection with the present invention, it 30 has been discovered that when these common contaminants are eliminated from the lead, and copper alloyed with the lead in the proportions indicated, bismuth in controlled amounts is actually helpful in the matter of corrosion resistance, whereas it does not adversely affect the creep properties of the alloy.

It has been found, in connection with the 35 present invention, that the presence of small amounts of bismuth, but not exceeding 0.0225% actually increases the corrosion resistance of the alloy because in the presence of such amounts of bismuth there is formed a protective coating of basic lead sulphate on the lead, which coating is very hard and dense, having ceramic characteristics. It is observed that such a coating is 40 formed between bismuth limits of 0.005% to 0.0225%, and with a copper content of from 0.04% to 0.08%. Above the above-specified maximum, bismuth is found to be definitely hurtful to 45 corrosion, as evidenced, among other facts, by the lowering of the flash point of the alloy.

The following tables show the specifications and physical properties of the improved lead of 50 the present invention with other grades of com- 55

mercial leads. In the tables, the lead indicated as "Grade I corroding" refers to the grade of lead which is usually employed for the production of lead pigments, such as white lead; "Grade II chemical" refers to the grade of lead commonly used where high sulphuric acid corrosion resistance is an essential characteristic, such as, for example, in the lead which is used for the lead chambers of sulphuric acid production; "Grade III common" is the usual commercial lead employed throughout the arts for the production of pipes, solder, and the more common usages for lead.

It is believed that the substantially complete elimination of all impurities from the lead which detract from the creep resistance properties of lead, particularly the silver being removed from the lead to a substantially complete elimination, produced in conjunction with the copper content of the alloy, the high resistance to creep, which effect is in no way offset by the controlled quantities of bismuth that are present in the alloy, so that this bismuth content as specified herein can be tolerated without any disadvantage either from the standpoint of lowered creep or lowered flash point; but additional bismuth over the

| 15                  | Improved acid<br>resisting lead<br>present<br>invention                             | A. S. T. M. specifications |                      |                                                           | 15          |
|---------------------|-------------------------------------------------------------------------------------|----------------------------|----------------------|-----------------------------------------------------------|-------------|
|                     |                                                                                     | Grade I cor-<br>roding     | Grade II<br>chemical | Grade III<br>common                                       |             |
| 20                  | Silver                                                                              | 0.002% max.                | 0.0015% max.         | { (0.020% max.<br>.002% min.<br>.080% max.<br>.040% min.) | 0.002% max. |
|                     | Copper                                                                              | .04-.08%                   | .0015% max.          | { .0025% max.<br>.015% max.<br>.005% max.                 | .0025% max. |
|                     | Copper + silver                                                                     |                            |                      |                                                           |             |
|                     | Arsenic                                                                             |                            |                      |                                                           |             |
|                     | Antimony + tin                                                                      |                            |                      |                                                           |             |
| 25                  | Arsenic, antimony and tin                                                           | .002% max.                 | .0015% max.          | .002% max.                                                | .015% max.  |
|                     | Zinc                                                                                | .001% max.                 | .0015% max.          | .001% max.                                                | .002% max.  |
|                     | Iron                                                                                | .0015% max.                | .002% max.           | .0015% max.                                               | .002% max.  |
|                     | Bismuth                                                                             | .02% max.                  | .05% max.            | .005% max.                                                | .15% max.   |
|                     | Nickel                                                                              |                            |                      |                                                           |             |
|                     | Cadmium                                                                             |                            |                      |                                                           |             |
| 30                  | Lead (by difference)                                                                | 99.90%                     | 99.94%               | 99.90%                                                    | 99.85%      |
| Physical properties |                                                                                     |                            |                      |                                                           |             |
|                     | Tensile strength lbs./sq. in.                                                       | 2250                       | 1700                 | 2300                                                      | 1700        |
| 35                  | Yield point lbs. per sq. in.                                                        | 950                        | 600                  | 1050                                                      | 600         |
|                     | % Elongation in 8 inches                                                            | 50                         | 50                   | 40                                                        | 50          |
|                     | Brinell hardness No.                                                                | 4.2                        | 4                    | 4.5                                                       | 4           |
|                     | Creep rate at 25° C. and 350 lbs./sq. in. Tensile load in inches per inch per year. | .003                       | .044                 | .0148                                                     | .044        |

In the above tests, the tensile determinations were conducted at a temperature of 25° C. and with a speed of .05 inch per inch per minute. The Brinell hardness values were determined by using a 10 mm. ball, with 100 kgm. loads at 30 seconds test period at 23° C. plus or minus five degrees, and are based on data obtained over a three year test period. The specimens were in the "as rolled" condition.

The present improved alloy possesses the following improved characteristics, among other properties which render it desirable for use wherever there may be required a composition of very high resistance to corrosion, and a high resistance to creep. In this connection it will be noted that the creep rate of the improved alloy is roughly only about one-fifth that of chemical lead, and by slightly more than one-tenth that of grade I corroding lead. The improved alloy is characterized by the following noteworthy properties: (1) Very high creep strength; (2) Exceptionally high resistance to acid corrosion; (3) Clean and free flowing, adaptable to the sound castings in slab mold and cylinder necessary to the proper production of rolled sheet and extruded pipe, free from foreign inclusions, lending itself to such melting operations where it is required that drossing be minimized; (4) Constant uniformity, lending itself to be worked with minimum variation of pressure on a die-block or roll-neck into accurate pipe and sheet; (5) Adaptable in sheet or pipe to the requirements of lead burners; (6) Being an ideal alloying base to which fabricators may add antimony, or other elements which conditions of use indicate it to be wise to incorporate for given conditions and purposes.

maximum specified herein adversely affects both the creep strength and the flash point, as has been indicated above.

The extremely high resistance to sulphuric acid corrosion exhibited by the present alloy may be attributed to the fact that there is produced on the alloy when in contact with sulphuric acid the hard, dense, extremely adherent protective coating which has been referred to above; and it is found that this coating, in the case of the present improved alloy, may be separated from the alloy only with a substantial amount of difficulty, and that this coating is substantially non-porous and impervious, so that a stable protective sheath of high density and of a higher degree of adherence is produced on the alloy; and this coating is not subject to deformation in view of the fact that the alloy is so highly resistant to creep.

Comparative tests regarding the formation of this protective coating show by way of illustrative example that the present alloy with the upper limits of bismuth tolerance will have produced upon it 0.132 gram of this protective coating per square inch of surface, whereas the chemical lead referred to above, with a bismuth content of 0.004%, and contain copper between 0.04% and 0.08%, will produce, under the same conditions, only 0.005 gram per square inch of surface of the protective coating. It is not known definitely to what this is attributable, but the fact so remains as indicated, it being thought that the presence of the bismuth in the indicated ranges facilitates the formation of this protective coating and imparts to it the dense and non-porous character thereof.

If the lead used should be bismuth free or contain bismuth below the herein-specified mini-

5      mum limit of 0.005%, the present improved properties may be secured by incorporating bismuth as well as copper into the lead base, until the herein-specified composition is reached. Except for the bismuth and copper as herein specified, the lead has been refined until it does not contain more than 0.0085% as the maximum of the combined non-lead constituents present therein.

10      What is claimed is:

10      1. A lead base alloy which is highly resistant to acid corrosion and possessing high creep resistance, which consists in fully refined lead having normal corrosion producing impurities removed to within harmless limits and containing from 0.04% to 0.08% copper and from 0.005% to 15      0.0225% of bismuth.

5      2. A lead base alloy containing 0.04 to 0.08% copper, 0.005 to 0.0225% bismuth, the balance being fully refined lead in which the silver content does not exceed 0.002% maximum, and having the commonly occurring corrosion producing impurities removed to within harmless limits.

10      3. A lead base alloy containing 0.04 to 0.08% copper, 0.005 to 0.0225% bismuth, the balance being fully refined lead in which the aggregate of contaminating impurities does not exceed substantially 0.008% as the maximum.

JESSE O. BETTERTON.  
ALBERT J. PHILLIPS.

15